

Oct. 15, 1940.

15. 1940. A. B. BROWN ET AL 2,217,727  
METHOD OF PREPARING HIGH MELTING POINT ASPHALT AND HIGH QUALITY  
BRIGHT STOCK FROM MIXED BASE RESIDUUM  
Filed June 9, 1938

Filed June 9, 1938



Inventors:-  
Arthur B. Brown  
Frank C. Croxton  
Bernard Ginsberg  
By Donald Payne  
Atty.

## UNITED STATES PATENT OFFICE

2,217,727

## METHOD OF PREPARING HIGH MELTING POINT ASPHALT AND HIGH QUALITY BRIGHT STOCK FROM MIXED BASE RESIDUUM

Arthur B. Brown and Frank C. Croxton, Hammond, Ind., and Bernard Ginsberg, Chicago, Ill., assignors to Standard Oil Company, Chicago, Ill., a corporation of Indiana

Application June 9, 1938, Serial No. 212,656

4 Claims. (Cl. 196—34)

This invention relates to bright stock manufacture and it pertains more particularly to the preparation of bright stock from mixed base crude residuums.

5 The object of our invention is to provide an improved method and means for making high quality bright stock from mixed base crude residuums. A further object is to provide a method and means for improving the efficiency 10 and effectiveness of acid treating residual oil stocks after a deasphalting step, whereby special asphalts can be produced without interfering with the acid treating and neutralization steps. A further object is to provide an improved method 15 and means for finishing an acid-treated filter stock to obtain petrolatums and bright stocks of improved cast, color stability and oxidation stability. Other objects will be apparent as the detailed description of the invention proceeds.

20 In the operation of the deasphalting plant at Whiting, Indiana, it was discovered that the amount of propane admixed with the oil during the acid treating step had a profound effect on the neutralizing and finishing steps. When operating with a propane-to-oil ratio below 3:1 it was found that the sour oil could not be effectively neutralized, even when excess caustic and intimate mixing was employed. This phenomena is 25 unexplainable in the light of our present knowledge and experience, but it is evident that the propane has some effect in the acid treating step other than that of a simple diluent or thinner.

The neutralization difficulty is not, as might 30 be expected, a function of the amount of acid used,—it is a function of the propane ratio during the acid-treating step. However, the amount of acid used is important from the standpoint of color stability. If large amounts of acid are employed the oil requires little or no clay to 35 meet color specifications, but such excessively treated oils are not stable against oxidation, and they tend to go off color on standing. We have found that not only the propane ratio, but also the amount of acid used must be regulated with- 40 in close limits, and that the finishing with clay must also be within certain limits if a stable, high quality bright stock is to be produced.

In practicing our invention we regulate the 45 propane ratio in the deasphalting step to produce asphalt of the desired melting point, penetration, etc. Such ratios may, for instance, be in the range of 2:1 to about 4:1. Subsequent to the deasphalting step and prior to the acid-treating step we add sufficient propane (if addition is 50 necessary) to bring the propane-to-oil ratio up

to at least 3:1, and preferably to 3.5:1 or more. The amount of acid should be sufficient to decolorize the oil only partially, and we have found that .25 to .3 pound of 93% sulfuric acid (or its equivalent) per gallon of original charging stock 5 meets this requirement when deasphalting is effected in about 3 to 4 volumes of propane at about 90° to 115° F., preferably at about 110° F. When lesser amounts of propane are employed in the deasphalting step the amount of acid required 10 may be increased to about .3 to .7 pound per gallon of oil. The amount of acid should be regulated so that in the claying step a filter yield of about 400 to 1000, preferably about 600 to 700 gallons per ton is obtained when using average 15 clay (this may be increased to 1500 gallons with new No. 1 clay). This amount of claying is essential for color and oxidation stability. We prefer to strain the oil through a spent filter prior to the dewaxing or cold settling step, and 20 finally to percolate the wax-free oil or petrolatum in a fresh filter at about 100 to 180° F.

Another feature of our invention, particularly 25 when it is applied to the refining of petrolatum, is our method of handling and eliminating "sludge pepper." When heavy oils or petrolatums are acid-treated in propane we have found that the treated product tends to suspend a "sludge pepper" which has to be removed before proper neutralization can be effected. We have 30 discovered that this "sludge pepper" may be removed by further settling if sufficient propane diluent is employed and sufficient settling time is allowed. Our method includes the provision of a "sludge pepper" settling step with a propane-to-oil ratio of at least 3.5:1 and in a settling zone of the type used for deasphalting or caustic settling. 35

The invention will be more clearly understood 40 from the following detailed description read in connection with the accompanying drawing which forms a part of this specification and which illustrates a flow diagram of our improved system for bright stock manufacture.

In our preferred embodiment we will describe 45 the preparation of bright stock from a Mid-Continent residuum reduced to about 20% bottoms and having a viscosity of about 350 to 400 seconds Saybolt at 210° F. It should be understood, however, that the invention is equally applicable to other charging stocks and to oils of widely varying composition.

A Mid-Continent reduced crude having a viscosity of about 365 to 370 seconds Saybolt at 55

- 210° F. is charged to the system through line 10 by means of pump 11 and is admixed with about 2½ volumes of propane from storage tank 12, pump 13 and line 14. This mixture is heated in 6 exchanger or heater 15 to a temperature of about 90° to 115° F., preferably about 100° F. to 110° F. and then introduced into asphalt settler 16 which is maintained at about 200 to 350 pounds pressure,—sufficient to prevent substantial vaporization. With this low propane ratio a 10 high melting asphalt of low penetration is separated out and withdrawn from the base of the settler through line 17 to a conventional asphalt depropanizer system.
- 15 The propane soluble fraction from the asphalt settler is withdrawn through line 18 to first acid sludge settler 19 but before it is introduced into the settler it is admixed with enough propane from line 20 to bring the propane-to-oil ratio up 20 to at least 3:1, and preferably to about 3.5:1. Instead of using fresh acid at this point we introduce cycle sludge through line 21 from the second acid sludge settler. The intimate mixture of deasphalted oil, propane and cycle sludge passes 23 down through the funnel-like center portion 22 of the first acid sludge settler into the quiescent zone in the lower part of the settler. Sludge is withdrawn from the base of the settler through line 23 to a conventional sludge depropanizer and 30 hydrolyzer. Sour oil from the upper part of the quiescent zone is withdrawn through line 24 to the upper part of second acid sludge settler 25. The fresh acid is introduced through line 26 preferably in amounts of about .2 to .5 pound of 93% 35 acid (or equivalent amounts of 98% acid, etc.) per gallon of original oil charged. The amount of acid in all cases should be so regulated that the oil can be finished to the desired color with a percolation yield of about 400 to 1000 gallons per ton 40 of average clay. It may also be desirable to add additional propane to line 24 through line 27, particularly if the propane ratio was low in the first acid sludge settler. It is most important that the propane-to-oil ratio in the second settler be at least 3 or 3½:1.
- 45 The sludge from the second settler is recycled through line 21 to line 18, as hereinabove described. If the sour oil from the upper part of the quiescent zone in the second settler is substantially free of "sludge pepper", it is withdrawn through line 28, admixed with caustic from line 29, and introduced into caustic settler 30. The amount of caustic will vary with different stocks and amounts of acid used, but we usually employ 50 about .035 pound per gallon (based on original oil charged) in the form of a 3% solution of sodium hydroxide. The used caustic solution is withdrawn from the base of the settler through line 31, and the neutralized oil is withdrawn 55 through lines 32 and 33 to propane still 34. Propane is removed from the top of the still through line 35 and recovered for reuse. Depropanized oil is withdrawn through line 36 to depropanized filter stock storage tank 37.
- 60 Filter stock from tank 37 is withdrawn by pump 38 and admixed with light naphtha withdrawn from tank 39 by pump 40, the blend of naphtha and filter stock being introduced through lines 41 and 42 to the top of a used clay 65 filter 43. The purpose of passing the solution through the used filter is to strain out certain color bodies and impurities, thereby improving the quality of the petrolatum to be later separated. The filter stock solution from used filter 70 43 is withdrawn through lines 44 and 45 to cold

settling tank 46 wherein the solution is gradually chilled to low temperatures for the settling of the petrolatum. Clear wax-free oil is withdrawn from the settling tank through line 47 to dewaxed solution storage tank 48, and the petrolatum is withdrawn from the base of the cold settler through line 49.

Dewaxed solution from tank 48 is next passed through line 50, heater 51 and line 52 to fresh clay filter 53 where it is percolated through clay 10 at about 100 to 180° F., preferably at about 110° F. to give a yield of about 400 to 1000 gallons per ton, preferably about 500 to 700 gallons per ton. From this clay filter the oil is passed through lines 54, 55 and 56 to naphtha-reducing still 57, 15 the naphtha being returned through line 58 and condenser 59 to naphtha storage tank 39, and the finished bright stock being withdrawn through line 60 to storage tank 61.

20 After settler 46 has been charged, as hereinabove described, the clay in filter 43 is revivified and/or fresh clay is added to this filter. Clay filter 53 now becomes the spent filter and the naphtha filter stock solution from line 41 is charged through lines 41 and 62 into spent filter 53 for 25 the straining step. The strained oil is withdrawn through lines 54 and 53, 44 and 64 to cold settling tank 65. After the solution has been chilled and settled in this tank the clear solution is withdrawn to dewaxed solution tank 48 through line 30 66 and the petrolatum is withdrawn from the base of the settler through line 67. The dewaxed solution now passes through line 50, heater 51 and line 68 to fresh filter 43, the clayed solution 35 being withdrawn through lines 69 and 56 to the naphtha-reducing still hereinabove described.

40 The straining, cold settling and filtering operations hereinabove described are designed for use in low pressure equipment. When high pressure equipment is available the use of naphtha may be entirely avoided and the neutralized oil from caustic settler 30 may be passed directly through lines 32, 10, 41 and 42 for straining in filter 43, or lines 32, 10, 41 and 62 for straining in clay filter 53. Somewhat higher filter yields may be obtained by the straining and subsequent filtration in propane solution, but here again the temperature should be maintained at about 100 to 110° F. for maximum efficiency.

45 When the propane is thus left in the solution the solidified petrolatum may be removed by filtration, instead of settling, in a conventional propane dewaxing filter, either before or after percolation.

50 The improved process hereinabove described produces a bright stock of excellent cast, an N. P. A. color of about 5 to 8, a 10° F. pour, 525 to 535° F. flash, and a viscosity of about 180 to 185 seconds Saybolt at 210° F. The bright stock is also stable against oxidation and color formation and is characterized by a low carbon residue and an acidity which is so low that it is negligible.

55 By regulating the propane ratio in the acid treating step subsequent to the deasphalting step, we have made it possible to use low propane ratios in the deasphalting step without interfering with the acid treating and neutralization steps. This enables the production of high quality asphalts in addition to the high quality bright stocks.

60 By operating at about 100-115° F. on a 20% M. C. residuum with a propane ratio lower than 3:1 we can produce an asphalt with a melting point above 170° F. and a penetration at 77° F. of less than 5. By blending this hard asphalt 75

with oxidized residuums, pressure tars, extract materials, and blending oils we can obtain high quality asphalts for all purposes.—asphalts of good temperature—ductility characteristics, high 5 solubility in carbon disulphide and benzol and any desired penetration and softening point characteristics.

By operating with longer residuums and at higher temperatures we can produce asphalts of 10 lower softening points, higher penetration, and good temperature susceptibility. No matter what conditions are used in the deasphalting step, as long as the proper propane ratio is maintained 15 in the acid treating step, neutralization can be easily effected.

When petrolatums or heavy oils are acid-treated it sometimes happens that the sour oil from the second settler contains appreciable amounts of "sludge pepper" which is suspended 20 or emulsified in the sour oil and which, unless it is removed, seriously impairs the quality of the finished oil or petrolatum. We have discovered that this "pepper" can best be removed by increasing the propane ratio to at least 3.5:1 25 and settling the pepper in a drum of the type used for settling asphalt and used caustic. If the asphalt settler is available this vessel may be used for the "pepper settle" and further equipment (except for the necessary lines, valves, 30 pumps, etc.) will not be necessary. We may, however, close the valve in line 28 and pass the sour oil or petrolatum thru line 71 to pepper settler 72, additional propane being introduced thru line 73 if necessary. The sludge pepper is 35 settled and withdrawn thru line 74 and may be depropanized and hydrolyzed with the material from line 23. The pepper-free oil or petrolatum is returned by line 75 to the caustic mixer and thence to caustic settler 30, as hereinabove de- 40 scribed.

Thus, the propane-to-oil ratio should be at least 3:1 in the acid treating step, but if in this step a sludge pepper is suspended in the oil, additional propane may be added and this pepper 45 settled out before the neutralization and further finishing steps. While we have described in de-

tail a preferred embodiment of our invention, it should be understood that we do not limit ourselves to any of said details except as defined by the following claims, which should be construed as broadly as the prior art will permit. 5

We claim:

1. The method of separately obtaining high melting point asphalt and high quality bright stock from mixed base crude residuums which comprises deasphalting said residuum with a propane-to-residuum ratio of less than 3:1 at a temperature of about 90 to 115° F., adding enough propane to the deasphalting oil to increase the propane-to-oil ratio to at least 3:1, treating the oil in this propane solution with acid at a temperature of about 90 to 110° F. with an amount of acid of about .2 to .7 pound of 93%-98% sulfuric acid per gallon of oil, neutralizing the sour oil and filtering the neutralized oil through clay at about 100 to 180° F. to obtain clay yields of 20 about 400 to 1000 gallons per ton of ordinary clay. 15

2. The method of claim 1 which includes the further step of dewaxing the neutralized oil prior to the final filtering through clay.

3. The method of claim 1 which includes the 25 steps of depropanizing the neutralized oil, mixing the depropanized oil with naphtha, straining the naphtha solution through a spent filter, dewaxing the strained naphtha solution, and subjecting the dewaxed solution to the filtration step 30 at about 100 to 180° F. to obtain clay yields of about 400 to 1000 gallons per ton of average clay. 35

4. The method of obtaining high melting point low penetration asphalts and high quality bright stocks which comprises deasphalting a mixed base residuum with a propane-to-residuum ratio less than 3:1, adding additional propane to the deasphalting oil to bring the propane-to-oil ratio to about 3:1 to 3.5:1, acid-treating the oil in the resulting propane solution with about .25 to .7 40 pound of 90% to 100% sulfuric acid per gallon of oil treated, neutralizing the acid-treated oil and treating said oil with clay.

ARTHUR B. BROWN.

FRANK C. CROXTON. 45  
BERNARD GINSBERG.